

## UNITED STATES PATENT OFFICE

1,961,468

## SINTERED ALLOY

Richard R. Walter, Starnberg, Germany

No Drawing. Application December 4, 1930,  
Serial No. 499,979. In Germany January 3,  
1930

## 7 Claims. (Cl. 75—1)

My invention pertains to a sintered alloy.

According to the specific exemplification of my invention, the exceptionally hard double carbide of chromium-tungsten ( $3\text{Cr}_3\text{C}_2\text{W}_2\text{C}$ ) constitutes the primarily effective constituent. In consequence of the difficulty of reducing chromium with hydrogen, that metal has hitherto been obtained by melting under an arc, but such a degree of brittleness thereby resulted that it was hitherto impossible to make technical use of the solidified complex carbide resulting from the melt.

However the resulting brittleness makes possible the attainment of an adequate degree of diminution to finest powdered form whereby to fabricate pieces formed as desired by means of pressing and subsequent sintering. The sintering temperature is fortuitously reduced in a manner by itself long known through the admixture of suitable metals, in order to avoid a new crystallization occurrence on the part of the carbides. The metals of the iron and chromium groups are adapted for that purpose, either singly or several together. The attainment of the most favorable relation of hardness and toughness is a matter of suitable selection according to the particular purpose of use.

Even small percentages of the metals of the iron group are adequate to effect cementation of the double carbide, for instance, three per cent (3%) nickel or one per cent (1%) iron and three per cent (3%) cobalt. Generally, the toughness increases and the hardness decreases as more auxiliary metals are added. If besides metals of the iron group one also selects from those of the chromium group, for example, cobalt and tungsten or cobalt and tungsten and chromium, larger quantities of these (approaching 50%) may be added with due consideration of toughness so as to obtain alloys which are adequately hard for many purposes and which are distinguished by reason of their great resistance to wear and corrosion.

It is also possible advantageously to replace a portion of the metals of the iron and chromium groups with their carbides or carbonitrides, so substituting for either one or several together. The tungsten carbides  $\text{W}_2\text{C}$  or  $\text{WC}$  or the nitrogen-inclusive combination  $\text{W}_x\text{C}_x\text{N}_y$  are especially adapted as such substitutes because as much as sixty per cent (60%) of them with reference to the total mass may be added together with a required minimum of about three per cent (3%) of pure metal for cementing the whole through sintering.

The following are cited as alloys embracing my invention:

| Per cent |   |                                                   |
|----------|---|---------------------------------------------------|
| 92       | — | ( $3\text{Cr}_3\text{C}_2\text{W}_2\text{C}$ ) 60 |
| 6        | — | Co                                                |
| 2        | — | Fe                                                |

or

|    |   |                                           |
|----|---|-------------------------------------------|
| 35 | — | ( $3\text{Cr}_3\text{C}_2\text{W}_2$ ) 65 |
| 35 | — | WC                                        |
| 10 | — | WCN (with 2% N)                           |
| 10 | — | Co                                        |
| 10 | — | W                                         |

These alloys serve manifold purposes, where-  
ever there is a demand for great resistance  
against wear or corrosion. The group with the  
greater auxiliary metal content are especially  
adapted for severely taxed machine parts as for  
instance, valves subjected to high pressure or  
high temperatures; moreover, because capable  
of taking on a high polish they are well suited  
for use on delicate measuring instruments, surgical  
instruments etc. The alloys with high car-  
bide content are best suited for cutting tools or  
as diamond substitutes on earth drilling tools.

For all the named or similar purposes the most  
favorable proportions of the ingredients are to  
be selected within the stated limits according  
to which the content of  $3\text{Cr}_3\text{C}_2\text{W}_2\text{C}$  should not  
be less than about thirty per cent (30%) of the  
total alloy.

I claim:

1. A sintered alloy comprising 30-97% of a  
chromium-tungsten double carbonaceous com- 90  
pound having the formula  $3\text{Cr}_3\text{C}_2\text{W}_2\text{C}$ , from 1  
to 60% of a carbonaceous compound of a metal  
of the sixth periodic series, a larger per cent of  
the latter being used with a lesser per cent of the  
former, and at least one metal of the iron or chro- 95  
mium group, the recited constituents forming  
substantially the entire content.

2. A sintered alloy comprising 30-97% of the  
chromium-tungsten double carbide having the  
formula  $3\text{Cr}_3\text{C}_2\text{W}_2\text{C}$ , from 1-50% metal of the 100  
chromium group, larger per cents of the latter  
being used with lesser per cents of the former  
and as remainder, metal of the iron group.

3. A sintered alloy comprising the chromium-  
tungsten double carbide having the formula 105  
 $3\text{Cr}_3\text{C}_2\text{W}_2\text{C}$  mixed with a carbonaceous compound  
of a metal of the chromium group and together  
constituting about 90% with at least 30% of the  
named double carbide and as remainder for cem-  
entation, about 10% of metal of the iron group. 110

4. A sintered alloy comprising the chromium-tungsten double carbide having the formula  $3Cr^3C^2.W^2C$  and an azotized carbide of tungsten, said double and azotized carbides together constituting about 90% and the former at least 30%, and about 10% cementation metal of the iron group.

5. A sintered alloy comprising 30-97% of the double chromium-tungsten carbide having the formula  $3Cr^3C^2.W^2C$  mixed with from 1-60% of a carbonaceous compound of a metal of the sixth periodic series, larger amounts of the latter being employed with lesser amounts of the former, and as remainder, metal of the iron group.

15 6. A sintered alloy comprising 30-97% of the

chromium-tungsten double carbide having the formula  $3Cr^3C^2.W^2C$  mixed with from 1-60% of a carbonaceous compound of tungsten the per cent of which increases when the per cent of the double carbide diminishes, and metal of the iron group as remainder.

7. A sintered alloy comprising about 80% of a mixture of the chromium-tungsten double carbide having the formula  $3Cr^3C^2.W^2C$  and of a carbonaceous compound of tungsten, the double carbide in said mixture being not less than 30%, and metal of the chromium group and metal of the iron group, which metals aggregate about 20%.

RICHARD R. WALTER. 90

|    |     |
|----|-----|
| 20 | 95  |
| 25 | 130 |
| 30 | 105 |
| 35 | 110 |
| 40 | 115 |
| 45 | 120 |
| 50 | 125 |
| 55 | 130 |
| 60 | 135 |
| 65 | 140 |
| 70 | 145 |
| 75 | 150 |